

# UNITED STATES PATENT OFFICE.

SIMON ADDE, OF GRÄNGESBERG, SWEDEN.

## PLASTIC EXPLOSIVE.

1,410,868.

Specification of Letters Patent. Patented Mar. 28, 1922.

No Drawing. Application filed January 26, 1917. Serial No. 144,680.

To all whom it may concern:

Be it known that I, SIMON ADDE, engineer, subject of the King of Sweden, residing at Grängesberg, Sweden, have invented certain new and useful Improvements in a Plastic Explosive, of which the following is a specification.

In my British Patent Nr. 13373 of 1912 I have described an explosive, the basic material of which consists of a "liquid nitrocompound" of an aromatic hydrocarbon gelatinized with nitrocellulose.

I have explained in that patent what I meant at that time by "liquid nitrocompound," namely the liquid mother lye remaining from the crystallization of the different nitro-derivatives of the said aromatic hydrocarbons. These mother lyes and residues from the distillation are, however, composed of the different isomeres of the said nitrocompounds and to a less part of higher nitromethane-derivatives, having a very low freezing point.

These mother lyes and residues from the distillation are composed of different nitro compounds and their chemical constitution is not fully known by the scientists.

Lately, however, the chemists have succeeded, by conducting the nitration process in special ways, in separating several nitro-derivatives from these mother lyes, said derivatives having an exact chemical constitution and of which some are solid while others have a fluid, oily consistence. Thus, for example, there are at present known six different mono-derivatives of the nitro-xylo. Amongst these derivatives two are solid, whereas the remaining four form oily fluids having a low freezing point.

I have found that all these fluid nitro-derivatives of the aromatic hydrocarbons are very good solvents of nitrocellulose, forming therewith a blasting gelatine, which has about the same properties as the well known gelatine of nitroglycerine and nitrocellulose, but differs from the latter in that it freezes only at a very low temperature even if a comparatively great percentage of nitroglycerine is added. Moreover, my new blasting gelatine has great stability and is very little sensible to heating and to mechanical shocks and the like.

In order to increase the plasticity of the gelatine thus facilitating its pressing through mouth-pieces of different diameters,

and also for the purpose of still further lowering the freezing point of the explosive, an addition of a small percentage of alcohol is very effective, I have found.

Especially methyl alcohol being an excellent solvent of nitrocellulose is suitable for the purpose.

The gelatine thus formed may then be mixed in the known manner with suitable substances yielding or containing oxygen, such as chlorates, perchlorates, or nitrates, and with combustibles (carbonaceous matters) until a doughy mass of about the same consistency as gelatinized dynamite is obtained.

I have found that the metals: aluminium, manganese, iron and silicon in finely divided state or finely divided alloys of some of the said metals are very effective.

Below are given some examples of the composition of my new explosive, intended for different blasting purposes.

### I. For blasting in open shaft mines.

|                                                                                                | Per cent. |
|------------------------------------------------------------------------------------------------|-----------|
| Perchlorate of ammonium                                                                        | 30 to 70  |
| Gelatinized:                                                                                   |           |
| Fluid derivatives of nitrated aromatic hydrocarbons with or without addition of nitroglycerine | 85        |
| Methyl alcohol                                                                                 | 20 to 40  |
| Nitrocellulose                                                                                 | 0.5 to 5  |
| Alloy of aluminium and silicon or of aluminium, manganese and silicon                          | 1 to 3    |
|                                                                                                | 90        |
|                                                                                                | 5 to 20   |

### II. For underground blasting.

| (a.)                                                                                  | Per cent. |
|---------------------------------------------------------------------------------------|-----------|
| Chlorate or perchlorate of sodium or potassium                                        | 30 to 70  |
| Gelatinized:                                                                          |           |
| Fluid derivatives of nitro - hydrocarbons, with or without addition of nitroglycerine | 100       |
| Methyl alcohol                                                                        | 20 to 40  |
| Nitrocellulose                                                                        | 0.5 to 5  |
| Alloy of manganese and aluminium or iron and aluminium                                | 1 to 3    |
| Wood-meal, charcoal or other carbonaceous material                                    | 5 to 20   |
|                                                                                       | 105       |
|                                                                                       | 0 to 5    |
|                                                                                       | 110       |

(b.)

|                                                                                             | Per cent.          |
|---------------------------------------------------------------------------------------------|--------------------|
| Perchlorate of ammonium or nitrate of ammonium-----                                         | 35 to 45           |
| 5 Nitrate of sodium or potassium Gelatinized:                                               | 25 to 35           |
| 10 Fluid derivatives of nitro hydrocarbons, with or without addition of nitroglycerine----- | 20 to 40           |
| 15 Ethyl alcohol preferably as extracted from sulphite waste lye-----                       | 0.5 to 2<br>1 to 3 |
| 20 Nitrocellulose-----                                                                      | 5 to 20            |
| Ferro-silicon or ferro-manganese-----                                                       | 0 to 5             |
| Wood-meal, charcoal or other carbonaceous material-----                                     | 0 to 5             |

The explosives described above may be pressed into long plastic strings which may be cut into cartridges of desired length in 25 the same way as gelatinized dynamite.

What I claim is:—

1. A plastic explosive compound of low freezing point, consisting solely of a liquid nitro-derivative of exact chemical constitution produced from an aromatic hydrocarbon, other than benzol and toluene, said nitro-derivative gelatinized with nitrocellulose.
2. A plastic explosive compound as specified in claim 1, in which nitroglycerin has 35 been added.
3. A plastic explosive compound, as specified in claim 1, in which a small percentage of alcohol has been added.
4. A plastic explosive compound, as specified in claim 1, in which a small percentage of methyl alcohol has been added.
5. A plastic explosive compound of low freezing point consisting solely of a liquid nitro-derivative of exact chemical constitution, produced from an aromatic hydrocarbon, other than benzol and toluene, said nitro-derivative gelatinized with nitro-cellulose, and materials containing oxygen and carbonaceous materials.
- 50 6. A plastic explosive compound as specified in claim 5, containing also nitroglycerin.

fied in claim 5, containing also nitroglycerin.

7. A plastic explosive compound as specified in claim 5, in which a small percentage of alcohol has been added.

8. A plastic explosive compound as specified in claim 5, containing also nitroglycerin and alcohol.

9. A plastic explosive compound as specified in claim 5, containing also in finely divided state a metal capable of increasing the temperature of the explosion.

10. A plastic explosive compound as specified in claim 5, containing also in finely divided state a metal capable of increasing the temperature of the explosion, and silicon.

11. A plastic explosive compound as specified in claim 5, containing also an alloy of metals capable of increasing the temperature of explosion.

12. A plastic explosive compound as specified in claim 5, containing also a metal capable of increasing the temperature of explosion, and silicon.

13. A plastic explosive compound as specified in claim 5, containing also alcohol, a metal, capable of increasing the temperature of explosion, and silicon.

14. A plastic explosive compound consisting solely of nitroxylen, gelatinized with nitro-cellulose.

15. A plastic explosive compound consisting solely of nitroxylen and nitroglycerin, gelatinized with nitro-cellulose.

16. A plastic explosive compound as specified in claim 14, containing also a small percentage of alcohol.

17. A plastic explosive compound as specified in claim 14, containing also oxygen yielding substances, carbonaceous materials, a metal capable of increasing the temperature of explosion, and silicon.

In testimony whereof I affix my signature in presence of two witnesses.

SIMON ADDE.

Witnesses:

HARRY ALBIHN,  
GUSTAF ALSON.